

1

3,252,914  
INHIBITING CORROSION OF COPPER- AND ZINC-  
CONTAINING METALS IN CONTACT WITH  
AERATED SOLUTIONS OF POLYPHOSPHATE  
SALTSJohn B. Braunwarth, Charanjit Rai, and Robert C. Kimble, all of Crystal Lake, Ill., assignors, by mesne assignments, to Union Oil Company of California, Los Angeles, Calif., a corporation of California  
No Drawing. Filed Apr. 13, 1962, Ser. No. 187,193  
13 Claims. (Cl. 252—137)

This invention relates to new and useful improvements in inhibiting the corrosion of copper-containing and zinc-containing metals in contact with aerated solutions containing polyphosphate salts, and more particularly to a novel detergent composition containing a cycloalkanone-aminobenzothiazole reaction product as a corrosion inhibitor.

Many surfaces are easily oxidized and corroded by contact with aerated aqueous solutions but usually can be protected by the incorporation of corrosion inhibitors in the solution. Various organic chemicals have been used as corrosion inhibitors for aerated solutions, such as amines, mercaptans, heterocyclic nitrogen compounds, substituted ureas and thioureas, etc. Commercial detergent compositions, however, have presented an especially severe problem because of their polyphosphate contents. The polyphosphates which are included in most detergent compositions tend to dissolve copper and zinc when contacted with those metals, either alone or in the form of their alloys such as galvanized iron, brass, bronze, etc. When aerated aqueous solutions containing polyphosphates are contacted with copper- or zinc-containing metals, there is a tendency for the metals to go into solution as metal-polyphosphate anions. Because the detergents prevent the deposition of protective films on the metal surfaces, little success has been realized heretofore in combatting the corrosiveness of aqueous detergent solutions.

It is therefore one object of this invention to provide a new and improved method for inhibiting the corrosion of copper- and zinc-containing metals when contacted by aerated solutions containing polyphosphate salts.

Another object of this invention is to provide a new and improved detergent composition containing a novel corrosion inhibitor for preventing corrosion of copper- and zinc-containing metals by polyphosphates in the detergent.

A feature of this invention is the provision of an improved process for inhibiting the corrosion of copper and zinc-containing metals in contact with aerated solutions containing polyphosphate salts wherein there is added to the solution about 0.005 to 0.20% wt. of a solution of the reaction product of a cycloalkanone and an aminobenzothiazole.

Another feature of this invention is the provision of an improved aqueous detergent solution containing water-soluble polyphosphate salts and from about 0.005 to about 0.20% wt. of a solution of the reaction product of a cycloalkanone and an aminobenzothiazole, sufficient to inhibit corrosion of copper- and zinc-containing metals when contacted by the solution.

Other objects and features of this invention will become apparent from time to time throughout the specification and claims as hereinafter related.

This invention is based upon our discovery that the corrosion of copper-containing and zinc-containing metals by aerated detergent solutions containing polyphosphate salts can be inhibited by adding to the solution (either separately or together with the detergent) a small amount, in the range of about 0.005 to 0.20% wt. of a solution of

2

the reaction product of a cycloalkanone and an amino-benzothiazole.

The reaction products which are used as corrosion inhibitors in accordance with this invention are prepared by mixing and heating an aminobenzothiazole and a cycloalkanone, or by reaction of a cycloalkanone with thiourea under acidic conditions. The aminobenzothiazoles used in the preparation of our corrosion inhibitor have the generic formula:



15 where



25 is a benzene or partially hydrogenated benzene nucleus, and R is lower alkyl or aryl; the cycloalkanones which are reacted with the amino-benzothiazoles to produce the novel corrosion inhibitors include C<sub>4</sub>—C<sub>10</sub> alkanones and alkyl and aryl derivatives thereof, such as cyclobutanone, cyclopentanone, cyclohexanone, cycloheptanone, cyclooctanone, cyclononanone, cyclodecanone, methylcyclopentanone, methylcyclohexanone, phenylcyclohexanone, benzocyclohexanone, etc. The cycloalkanones which can be used also include condensed derivatives of the cycloalkanones produced by acidic condensation, e.g., 2-35 cyclohexylidienyl cyclohexanone, 2-cyclopentylidienyl cyclopentanone, 2-cycloheptylidienyl cycloheptanone, etc.

40 A preferred method of preparation of these corrosion inhibitors is to reflux an aminobenzothiazole with a cycloalkanone for a period of about 1 to 3 hours to produce a syrupy reaction product. The reactants are preferably added in stoichiometric portions in accordance with the reaction,



55 where



65 is a cycloalkanone or substituted cycloalkanone.

Alternatively, certain of the corrosion inhibitors used herein can be prepared by essentially a one-step process by reaction of a cycloalkanone such as cyclohexanone with thiourea under acidic conditions. Under these conditions, a reaction takes place which produces a hydrogenated derivative of the thiazole-cycloalkanone reaction product, which in some cases contains a cycloalkylidene substituent on the cycloalkanone portion of the reaction product. In general, the reaction products which are used as corrosion inhibitors in accordance with this invention are mixtures containing as an active in-

redient at least one compound selected from the group consisting of:



and



where



is a radical selected from the group consisting of  $C_4$ – $C_{10}$  cycloalkylidene radicals and condensed derivatives thereof containing a  $C_4$ – $C_{10}$  cycloalkylidene substituent, and lower alkyl and aryl derivatives thereof.

The following non-limiting examples are illustrative of the scope of this invention.

*Example I*

In one experiment, 8.3 g. of 2-amino-4,5,6,7-tetrahydrobenzothiazole hydrochloride was mixed with 30 cc. of cyclohexanone. The mixture was refluxed for 3 hours. At the end of this reaction time, excess cyclohexanone was removed by distillation, leaving the product ready for use. The product obtained in this reaction was a mixture consisting of



and



The effectiveness of our corrosion inhibitor has been demonstrated by a series of experiments with aqueous solutions of a commercial detergent containing mixed aryl alkyl sulfonates, sodium tripolyphosphate, sodium sulfate, and other components. The detergent used in these experiments is a household detergent sold under the trademark Tide (product of Procter and Gamble, Inc.). First, a water solution of Tide was prepared in a concentration of 0.5 g. per 100 ml. water and divided into two flasks. Into one of the flasks there was added a sufficient amount of the reaction product of cyclohexanone and 2-amino-4,5,6,7-tetrahydrobenzothiazole to achieve a concentration of 0.1 g. per 100 ml. of solution. Then, two brass strips (1/2 inch x 3 inches) were immersed in the solution in each flask and air was bubbled through the solutions at a rate of 20–30 ml./min. for a period of 72 hours while the temperature was maintained at 70° C. The weight losses from the brass strips were as follows:

|              | Weight Loss, <sup>1</sup><br>(percent) | Corrosion Rate<br>(in./yr.) |
|--------------|----------------------------------------|-----------------------------|
| Control----- | 1.70                                   | 0.0682                      |
| Test-----    | 0.01                                   | 0.0006                      |

<sup>1</sup> Average of two coupons.

From these experiments it is seen that the corrosion inhibitor used with the detergent resulted in the reduction of more than 99% in corrosion rate.

*Example II*

To 15.2 g. of thiourea and 4 g. of hydrochloric acid was added 42 cc. of cyclohexanone. The mixture was refluxed for 3 hours and the product poured into warm aqueous ethanol. The crystalline material which appeared in 3 or 4 hours was filtered and dried. When this reaction product is added to a detergent solution containing water-soluble polyphosphate salts in a concentration of the additive in the range of about 0.005% to 0.20% wt. of the solution, the rate of corrosive attack of the solution on copper- and zinc-containing metals is decreased by about 90%.

*Example III*

To 25 g. of 2-aminobenzothiazole is added 30 cc. of cyclohexanone. The mixture is refluxed for 3 hours. Excess cyclohexanone is then removed by distillation leaving the product ready for use. The product obtained consists essentially of:



When this reaction product is incorporated into an aqueous detergent solution containing water-soluble polyphosphates in an inhibitor concentration in the range from about 0.005 to 0.20% wt. of the solution, the corrosivity of the solution toward zinc and copper containing metals is reduced by more than 90%.

*Example IV*

To 30 g. of 2-aminobenzothiazole is added 90 cc. of cyclohexanone and 4 g. of hydrochloric acid. The mixture is refluxed for 3 hours and excess cyclohexanone and acid are removed by distillation. The product obtained consists mainly of:



When this reaction product is incorporated into an aqueous detergent solution containing water-soluble polyphosphates in an inhibitor concentration of 0.005 to 0.20% wt. of the solution, the tendency of the solution to corrode copper- or zinc-containing metals is reduced by an amount in excess of 90%.

When other cycloalkanones are reacted with aminobenzothiazole (or hydrogenated derivatives thereof) reaction products are obtained within the scope of the general formula given above. Likewise, when other cycloalkanones are reacted with thiourea under acidic conditions, a mixed reaction product is obtained containing compounds within the general formula. When these reaction products are incorporated into an aqueous detergent solution containing water-soluble polyphosphates, in an inhibitor concentration in the range from about 0.005 to 0.20% wt. of the solution, the tendency of the solution to corrode copper- and zinc-containing metals is decreased by more than 90%. While the effectiveness of these corrosion inhibitors has been demonstrated primarily in connection with aerated solutions, it should be noted that a similar corrosion-inhibiting effect is obtained in the absence of aeration of the solution.

While we have described our invention fully and completely with special emphasis upon several preferred em-

bodiments of our invention, we wish it to be understood that within the scope of the appended claims this invention may be practiced otherwise than as specifically described herein.

The embodiments of the invention in which an exclusive 5 property or privilege is claimed are defined as follows:

1. A method of inhibiting the corrosion of copper- and zinc-containing metals in contact with aqueous, aerated 10 solutions of polyphosphate salts in amounts conducive to corrosion which consists essentially of adding to the solution a small amount, in the range of about 0.005 to 0.20% wt. of the solution, of the reaction product of stoichiometric quantities of a cycloalkanone selected from the group consisting of cyclobutanone, cyclopentanone, 15 cyclohexanone, cycloheptanone, cyclooctanone, cyclononanone, cyclodecanone, methylcyclopentanone, methylcyclohexanone, phenylcyclohexanone, benzocyclohexanone, 2 - cyclohexylidene cyclohexanone, 2 - cyclopentylidene cyclopentanone, 2-cycloheptylidene cycloheptanone, and an aminobenzothiazole selected from the 20 group consisting of



and



2. A method in accordance with claim 1 in which the reaction product is added in admixture with the polyphosphate salts.

3. A method in accordance with claim 1 in which said reaction product includes as an active ingredient at least one compound selected from the group consisting of:



and



where



is a radical selected from the group consisting of 2-cyclohexylidene cyclohexylidene, 2-cyclopentylidene cyclopentylidene, 2 - cycloheptylidene cycloheptylidene, C<sub>4</sub>-C<sub>10</sub> cycloalkylidene and methyl, phenyl and benzo derivatives thereof.

4. A method in accordance with claim 3 in which said active ingredient is



5. A method in accordance with claim 3 in which said active ingredient is



6. A method in accordance with claim 3 in which said active ingredient is



7. A method in accordance with claim 3 in which said active ingredient is



8. An aerated aqueous detergent solution of water 30 soluble polyphosphate salts in amounts conducive to corrosion, and a small amount, in the range from about 0.005 to 0.20% wt. of the solution, of the reaction product of stoichiometric quantities of a cycloalkanone selected from the group consisting of cyclobutanone, cyclopentanone, cyclohexanone, cycloheptanone, cyclooctanone, cyclononanone, cyclodecanone, methylcyclopentanone, methylcyclohexanone, phenylcyclohexanone, benzocyclohexanone, 2-cyclohexylidene cyclohexanone, 2-cyclopentylidene cyclopentanone, 2-cycloheptylidene cycloheptanone, and an aminobenzothiazole selected from the 40 group consisting of



and



55 9. The solution in accordance with claim 8 in which said reaction product includes as an active ingredient at least one compound selected from the group consisting of



where



is a radical selected from the group consisting of 2-cyclohexylidienyl cyclohexylidene, 2-cyclopentylidienyl cyclopentylidene, 2-cycloheptylidienyl cycloheptylidene,  $C_4-C_{10}$  cycloalkylidene and methyl, phenyl and benzo derivatives thereof.

10. The solution in accordance with claim 9 in which said active ingredient is



11. The solution in accordance with claim 9 in which said active ingredient is



12. The solution in accordance with claim 9 in which said active ingredient is



13. The solution in accordance with claim 9 in which said active ingredient is



References Cited by the Examiner

UNITED STATES PATENTS

|           |         |           |       |            |
|-----------|---------|-----------|-------|------------|
| 2,238,651 | 4/1941  | Keenen    | ----- | 252—394 XR |
| 2,618,603 | 11/1952 | Schaeffer | ----- | 252—137 XR |
| 2,618,605 | 11/1952 | Schaeffer | ----- | 252—137    |
| 3,062,612 | 11/1962 | Boucher   | ----- | 252—390 XR |

JULIUS GREENWALD, Primary Examiner.

W. E. SCHULZ, Assistant Examiner.